

Feb. 26, 1924.

1,484,669

V. PASTORE

HAIRCLOTH FABRIC

Filed July 20, 1920

Fig. 1



Fig. 2



Fig. 3



INVENTOR  
Vincent Pastore

## UNITED STATES PATENT OFFICE.

VINCENT PASTORE, OF NORWICH, CONNECTICUT.

## HAIRCLOTH FABRIC.

Application filed July 20, 1920. Serial No. 397,696.

*To all whom it may concern:*

Be it known that I, VINCENT PASTORE, a citizen of the United States, residing at Norwich, in the county of New London, in the State of Connecticut, have invented a certain new and useful Improvement in Haircloth Fabrics, of which the following is a specification, reference being had to the accompanying drawings.

10 This improvement relates to hair cloth of the type used commonly by tailors and others for stiffening garments, said cloth comprising usually a cotton warp and a filling of stiff hair, my present purpose being 15 to provide simple and inexpensive means for preventing the accidental disarrangement of the filling hairs with respect to the warp in the woven fabric.

In the building up of garments, particularly men's coats, hair cloth of the class referred to is commonly utilized for stiffening such garments and it is the common experience that the wearers of the garments are annoyed by the working loose of the 20 stiff filling hairs which, being as sharp as fine needles, readily prick through the cloth and must then be drawn out and thrown away. To overcome this objectionable action of the stiffening the cut ends of said 25 hairs are sometimes protected, and prevented from escaping, by binding the edges of the stiffening fabric but this involves an expenditure of time and material which it is desirable to avoid, especially in cheap clothing. My present purpose is to provide simple and cheap means in such stiffening cloth whereby the filling hairs are positively anchored in the warp and therefore said hairs 30 cannot escape and, with this desirable purpose in view, I have provided the fabric illustrated in the annexed drawings, in which the Figure 1 is a face view of one-half of the front of a coat showing also the stiffening fabric outlined thereon. Figure 2 is a relatively enlarged view of the 35 upper portion of said stiffening cloth and Figure 3 is a transverse sectional view of said cloth taken at the line 3—3 of said Figure 2.

Referring to these drawings, the letter *a* indicates a portion of a coat front and *b* denotes the portion of said front which is to be folded back along the dotted line *c* to provide the customary lapel. *d* denotes 40 a stiffening of hair cloth which may be of

any desired size and shape; as here shown it is designed to stiffen the front of the garment and particularly the shoulder and neck portions; the edge portion of said stiffening being partially overlapped and enclosed when the lapel portion is folded back and pressed down. The essential feature of my present improvement is in the novel construction of the hair cloth fabric, as I have already stated. The warp threads 45 of said fabric are indicated in the drawings by the letter *e* and the filling or weft by the letter *f*, the warp being cotton or other suitable material which is more or less flexible and the filling being of relatively stiffer material such as horse hair or bristles. Owing to the stiff, wiry nature of the filling such fabrics cannot be beaten up close enough in the weaving operation to crimp the filling and, as a result, the filling 50 hairs may be easily drawn out and, unless their cut ends are protected in some manner, said hairs work out through the garment fabric, as I have explained. In order to prevent such objectionable working out of 55 the hairs I subject the woven fabric to treatment which, in effect, cements the filling to the warp. This may be accomplished very cheaply and effectively by passing the fabric through a solution of white lead 60 which has been brought to a limpid consistency by the aid of turpentine, alcohol, benzine or the like, which readily saturates the fabric and, when dissipated by evaporation, leaves the hardened lead to operate 65 as a binder between the warp and filling without, however, objectionably stiffening the treated fabric.

In the Figure 3 of the drawings the binder of lead or other material, as the case may be, is denoted by the letter *g*.

The cost of thus treating the fabric is very small when compared with the resulting advantages and I find, by repeated practical use of such an improved fabric, that 100 it serves the desired purpose most satisfactorily.

The white lead wherever referred to in the specification refers to that type of base for paint which is known as the commercial white lead and is in the form of a paste and composed of a large percentage of white lead and a small percentage of linseed oil. The composition of the white lead for practical purposes is approximately 92% of 105

white lead mixed with approximately 8% cloth impregnated with commercial white of linseed oil.

Having thus described my invention, I claim:—

- 5 1. As a new article of manufacture, hair cloth and a cementitious paste formed of a commercial base for white paints for flexibly binding the warp and filling of the cloth together.
- 10 2. As a new article of manufacture, hair

cloth impregnated with commercial white lead as a binder.

3. A process of treating hair cloth to maintain the hairs in position in the cloth which comprises dissolving a commercial base of white lead in a readily evaporable solution, saturating the fabric with such solution and then evaporating the solution.

VINCENT PASTORE.

EXACT COPY